



US011499270B2

(12) **United States Patent**  
**Hernandez Rosario et al.**

(10) **Patent No.:** **US 11,499,270 B2**  
(45) **Date of Patent:** **Nov. 15, 2022**

(54) **PROTECTIVE BARRIER COATING FOR TUBES AND CORES**

(71) Applicant: **Sonoco Development, Inc.**, Hartsville, SC (US)

(72) Inventors: **Ismael Antonio Hernandez Rosario**, Florence, SC (US); **Aaron Edward Lintz**, Florence, SC (US); **Kevin Manly Kelley**, Hartsville, SC (US)

(73) Assignee: **Sonoco Development, Inc.**, Hartsville, SC (US)

(\*) Notice: Subject to any disclaimer, the term of this patent is extended or adjusted under 35 U.S.C. 154(b) by 37 days.

(21) Appl. No.: **17/175,272**

(22) Filed: **Feb. 12, 2021**

(65) **Prior Publication Data**

US 2021/0164164 A1 Jun. 3, 2021

**Related U.S. Application Data**

(63) Continuation of application No. 16/418,039, filed on May 21, 2019, now Pat. No. 10,941,523.

(60) Provisional application No. 62/677,282, filed on May 29, 2018.

(51) **Int. Cl.**

**D21H 19/84** (2006.01)

**D21H 19/40** (2006.01)

**D21H 19/16** (2006.01)

**D21H 27/30** (2006.01)

(52) **U.S. Cl.**

CPC ..... **D21H 19/84** (2013.01); **D21H 19/16** (2013.01); **D21H 19/40** (2013.01); **D21H 27/30** (2013.01)

(58) **Field of Classification Search**

None

See application file for complete search history.

(56) **References Cited**

**U.S. PATENT DOCUMENTS**

|                 |         |                   |
|-----------------|---------|-------------------|
| 4,855,354 A     | 8/1989  | Mohler et al.     |
| 5,144,056 A     | 9/1992  | Lina et al.       |
| 5,498,661 A     | 3/1996  | Hutter            |
| 6,066,373 A     | 5/2000  | Floyd, Jr. et al. |
| 6,123,753 A     | 9/2000  | Craig et al.      |
| 6,416,817 B1    | 7/2002  | Rangwalla et al.  |
| 9,751,721 B1    | 9/2017  | Hernandez         |
| 2005/0266166 A1 | 12/2005 | Halsey et al.     |
| 2007/0218292 A1 | 9/2007  | Shimada et al.    |
| 2010/0224817 A1 | 9/2010  | Jin               |
| 2011/0057069 A1 | 3/2011  | Hernandez et al.  |
| 2012/0285645 A1 | 11/2012 | Kusumi et al.     |

**FOREIGN PATENT DOCUMENTS**

|    |               |         |
|----|---------------|---------|
| JP | 2005188016 A  | 7/2005  |
| JP | 2010149474 A  | 7/2010  |
| KR | 0166171 B1    | 12/1998 |
| WO | 2016044880 A1 | 3/2016  |

*Primary Examiner* — Chinessa T. Golden

(74) *Attorney, Agent, or Firm* — von Briesen & Roper, s.c.

(57) **ABSTRACT**

A paperboard carrier suitable for use with textiles may include one or more strips of paperboard secured together to form a hollow tubular body, the body having an outer surface, and a coating covering some or all of the outer surface. The coating comprises a coating agent such as a silicon resin dispersed in a solvent such as isopropyl alcohol and little or no water. The coating may be applied to the outer surface by using a plurality spray nozzles arranged axially or circumferentially about the carrier.

**20 Claims, 5 Drawing Sheets**



**FIG. 1**



**FIG. 2**





**FIG. 4**



**FIG. 5**

## 1

PROTECTIVE BARRIER COATING FOR  
TUBES AND CORESCROSS REFERENCE TO RELATED  
APPLICATION

This application is a continuation of U.S. application Ser. No. 16/418,039, filed May 29, 2019. U.S. application Ser. No. 16/418,039 is incorporated here by reference in its entirety to provide continuity of disclosure.

## BACKGROUND

## Field of the Invention

This patent relates to cones and tubes for carrying wound materials. More specifically, this patent relates to cones and tubes having a protective barrier coating to prevent the transfer of chemicals between the tube or cone and the material wound into the tube or cone.

## Description Of The Related Art

Tubes and cones (hereinafter collectively referred to as "tubes" or "carriers") made of spirally wound paper often are used to hold wound materials such as sheet materials, carpet, yarn and other stand materials. The carriers may be custom made to satisfy a customer's needs, and vary greatly through special finishing processes, chemical treatments, paper stock and adhesives. The degree of crush, beam and torque strengths can be controlled to customer specifications. Carriers can be made to resist moisture, oil, chemicals, heat and abrasion.

Carriers used for carrying yarn and other strand materials typically have a smooth surface. However, they can be embossed, scored, grooved, perforated, polished, flocked, waxed and ground to provide desired surface characteristics. Tubes can be made with special inside or outside plies and can be made plain, colored or printed with stripes and other designs. Alternatively, colored bands can be applied to one or both ends for identification purposes. Labels applied to the inside can be used for further identification. Tube ends can be cut, crimped, rounded, beveled or otherwise finished to the customer's order.

Spirally wound tubes are particularly useful for carrying textiles, including yarn and thread. The tube can be made of plain paper stock and, for the outermost ply, a colored paper stock or a paper stock with a pattern or design. The ends typically are rounded.

Yarns and other textiles are frequently coated with chemicals to provide a desired characteristic or property for downstream processing, such as low friction or anti-static. There have been cases of chemical transfer from the yarn to the tube carrier during or after winding. As these chemicals transfer to the tube, the downstream processing can deteriorate.

One initial solution to the problem of chemical transfer involved using specialty coverings on the surface of the tubes, such as parchment or greaseproof papers. However, there are drawbacks to using coverings. First, the covering is typically wound in a helical fashion onto the paperboard core, and hence there may be gaps between each wrap of the specialty paper around the paperboard core. Alternatively, the specialty paper may be overlapped on each wrap, but this creates undesirable bumps along the surface of the paperboard core at the overlapping joints. Second, in order to recycle specialty paper-covered paperboard cores, either the

## 2

specialty paper must be removed prior to recycling, or else costly sorting and filtering equipment must be incorporated into the recycling machinery. Finally, as the textile manufacturers develop more sophisticated and/or aggressive coatings for their textiles, these coverings sometimes are not sufficient in preventing the chemical transfer from the textile to the tube.

The present disclosure addresses these drawbacks.

## 10 SUMMARY OF THE INVENTION

The present disclosure relates to a paperboard carrier suitable for use with textiles.

In one aspect a paperboard carrier suitable for use in 15 winding a material thereon and including a barrier coating is provided. The carrier may include one or more strips of paperboard wrapped about an axis and secured together to form an elongate structure, the elongate structure defining an outer surface. The coating covers some or all of the outer 20 surface. The coating comprises a coating agent dispersed in a solvent and little or no water. The coating agent may be a fluorourethane copolymer, a silicone resin, a fluoroalkyl acrylate copolymer emulsion or any other suitable coating agent. The solvent may be acetone, isopropyl alcohol (IPA), n-butyl acetate, mineral spirits, or other suitable solvent. The coating may be applied to the outer surface by using a variety of methods, such as applying with a kiss roll, spraying, or brushing. The coating is not heat cured.

## 30 THE DRAWINGS

FIG. 1 is a perspective view of a tube.

FIG. 2 is a perspective view of a tube carrying wound strand material.

FIG. 3 is a flowchart of a method of making a tube according to the disclosure.

FIG. 4 is a schematic depiction of a tube being formed and cut.

FIG. 5 is a schematic depiction of a tube being coated with 40 a protective barrier coating.

35 DETAILED DESCRIPTION OF THE  
INVENTION

While this invention may be embodied in many forms, there is shown in the drawings and will herein be described in detail one or more embodiments with the understanding that this disclosure is to be considered an exemplification of the principles of the invention and is not intended to limit the invention to the illustrated embodiments.

The present disclosure relates to using a coating on the paperboard tube to prevent yarn oil or other chemicals from migrating into paperboard core. As used herein, the term "coating" refers to a substance that is applied in a liquid 55 form, as opposed to a solid.

## The Carrier 10

FIG. 1 is a perspective view of a carrier 10, sometimes referred to as a tube or core. The carrier 10 may comprise a hollow cylindrical body 12 having an outer surface 14, an 60 inner surface 15, opposing ends 16 and a middle section 18 between the ends 16. The carrier 10 also has an axial dimension extending from one end 16 to the other end 16 and a radial dimension extending radially outward from an axis A. The carrier 10 may be used to carry stand material, such as yarn, or sheet material such as fabric, foil or paper. Typical tubes 10 for carrying textiles may have an outer diameter of three to four inches (7.62 to 10.16 cm) and may

be about one foot (30.48 cm) in axial length, although the tubes **10** may be any suitable dimensions depending on the application. The carrier **10** may be made from any suitable material or combination of materials, including paper, plastic or even metal foil.

The carrier **10** may comprise a tubular shape, as illustrated in FIG. 1. In alternate embodiments the carrier **10** instead take the form of a conical shape, or other shapes depending on the specific application. The carrier **10** in FIG. 1 is illustrated as a spirally wound carrier **10** in which strips of material are helically wrapped, but cores in accordance with the invention can instead be convolutedly wrapped.

FIG. 2 is a perspective view of a carrier **10** carrying wound strand material **20**, for example, yarn. If the carrier **10** is to be used to carry a textile, the carrier **10** may sold to the textile manufacturer who then winds their product **20** on the carrier **10**.

#### Method of Making the Carrier **10**

FIG. 3 illustrates an embodiment of a method **100** of manufacturing a carrier **10** according to this disclosure.

##### Winding

In a first operation **102**, the method **100** comprises winding one or more strips of paperboard about an axis (A) to form an elongate structure having a body **12**. The body **12** has an outer surface **14** facing away from the axis (A) and adapted to receive ("carry") a wound material thereon, and an inner surface **15** facing the axis (A). Each of the plurality of annular strips may be applied individually.

The winding operation **102** may be achieved through conventional means, such as that described in co-owned U.S. Patent Publication No. 2005/0260365, which now will be briefly described with reference to FIG. 4. The illustrated winding apparatus **22** is a spiral winding apparatus for making spirally or helically wound tubes **10**, one of which is depicted in FIG. 1. This particular winding apparatus **22** is used to manufacture a 4-ply tube, but the principles pertaining to the 4-ply tube are equally applicable to tubes having any number of plies. The winding apparatus **22** includes a cylindrical mandrel **24** whose diameter is selected to match the desired inside diameter of the tubes **10** to be manufactured, a winding belt **26** arranged to wrap about the tube formed on the mandrel **24** and about a pair of rotating drums **28** that drive the belt **26** such that the belt **26** advances the tube along the mandrel **24** in screw fashion at a substantially constant pitch. Four strips **32a**, **32b**, **32c**, and **32d** are drawn from respective supply rolls (not shown) and are advanced toward the mandrel **24** and are sequentially wrapped about the mandrel **24** in radially superposed fashion, one atop another. The winding apparatus **22** may include adhesive applicators **34b**, **34c**, and **34d** for applying adhesive to each of strips **32b**, **32c**, and **32d**, respectively. The adhesive applicators are structured and arranged so as to apply the adhesive to each of strips **32b**, **32c**, and **32d**, such as in the partial-coverage patterns **36b** and **36d** shown in FIG. 4.

##### Cutting

In a second operation **104**, the elongate structure is cut to create a tube **10** having opposing first and second ends **16** and desirable axial length. Referring again to FIG. 4, a cutting station **30** downstream of the winding apparatus may be used to cut the continuous tube formed on the mandrel **24** into individual tubes **10**.

##### Coating

In a third operation **106**, the method **100** comprises applying a coating **50** onto the outer surface **14** of the tube or carrier **10** in predetermined regions. The coating operation **106** may take a number of different forms.

##### Coating Application Methods

For example, the step **106** of applying a coating **50** may comprise roll-coating a coating **50** onto the outer surface **14** of the carrier **10**. The step of roll-coating may comprise rotating the paperboard carrier **10** against a rotating cylinder that is partially immersed in the coating **50**.

Alternatively, the coating **50** may be applied onto the outer surface **14** using a wick, brush, or the like.

Preferably the coating **50** is applied to the outer surface **14** by spraying. FIG. 5 is a schematic depiction of a carrier **10** being spray coated.

Number of Layers. The step **106** of applying the coating **50** may comprise applying a single layer of the coating **50**. Alternatively, the step **106** of applying the coating **50** comprises applying a plurality of layers of the coating **50**.

Uninterrupted coating **50**. The step **106** of applying a coating **50** may further comprise creating a substantially uninterrupted coating **50** on the outer surface **14**. In this regard, a paperboard carrier **10** with a coating **50** may avoid overlapping joints or gaps associated with use of a specialty covering. The coating **50** may comprise and may be applied as a plurality of annular bands arranged along the carrier **10** in the axial direction such that the coating **50** is uninterrupted.

The coating operation **106** may be accomplished by coating the elongated, uncut tube prior to it being advanced to the cutting station, or to the finished cut carrier **10**.

##### Alternative Method of Making the Carrier **10**

Instead of coating the elongated, uncut tube or finished cut carrier **10**, the coating **50** may be applied to the paperboard strips or plies **32** used to make the carrier **10**. For example, the step **106** of applying the coating **50** may comprise coating the radially outer surface of at least one of the one or more strips **32** prior to the step **102** of winding the one or more strips **32** about the mandrel **24**.

The coating **50** may be dried or otherwise cured. Multiple layers of the coating **50** may be sequentially applied and cured individually. However, it is expected that the diluted composition of the coating **50** will eliminate the need for heated curing to achieve the desired barrier properties.

##### The Coating Composition

The liquid coating **50** comprises a coating agent, a solvent and little or no water. The coating agent may be dispersed in the solvent.

The coating agent may be a fluorourethane copolymer, a silicone resin, a fluoroalkyl acrylate copolymer emulsion or any other suitable coating agent.

The solvent may be acetone, isopropyl alcohol (IPA), methyl alcohol, n-butyl acetate, mineral spirits, or other suitable solvent.

In one formulation the coating **50** is a silicone formulation such as a silicone resin dispersed in isopropyl alcohol (IPA) in relative amounts that achieve desirable flow and spray characteristics, with little or no water. The concentration of the silicone resin in the IPA may range from 1 to 10 percent or higher. This chemical formulation allows for very fast curing times in air, eliminating the need for heated drying.

This chemical formulation also allows the tube manufacturer to apply the coating **50** very close to the packing station without causing dimensional instability of the tubes. Finally, this formulation enables the tube manufacturer to print on the cores during the finishing process, applying the coating **50** and packing the tubes in a single unit.

The silicone resin may be a reactive silicone resin, that is, one that produces a durable moisture barrier when applied to a substrate. The silicone resin may comprise a siloxane. More particularly, the silicone resin may comprise silicone

resin and octamethylcyclotetrasiloxane. Still more particularly, the silicone resin may comprise 50% silicone resin and 50% octamethylcyclotetrasiloxane.

In another formulation the coating **50** comprises about 50% fluoroalkyl acrylate copolymer emulsion and about 50% methyl alcohol. The coating **50** may be a predetermined color used to identify a type of tube.

The coating **50** may achieve a desired barrier characteristic. For example, the coating **50** may provide superior oil or chemical resistance.

The concentration of the coating agent in the solvent can be tailored to the production equipment and the textile coatings that the customer (such as a textile manufacturer) might use or develop. Should the customer develop a more aggressive textile coating, the tube manufacturer can increase the concentration of the tube coating material to obtain the desired barrier properties.

#### System for Making a Coated Carrier **10**

In accordance with this disclosure a system **200** for making a coated carrier **10** is provided. Referring to FIG. 5, a completed, cut cylindrical paperboard carrier **10** is shown. The carrier **10** comprises one or more strips **32** of paperboard that have been wrapped around a mandrel and secured together to form an elongate structure, then cut to a desired length. The completed carrier **10** is an elongate structure defining a central axis (A) and having an outer surface **14** and an inner surface **15**.

The system **200** comprises a plurality of spray nozzles **40** and a controller **210**. The spray nozzles **40** apply the coating **50** onto the outer surface **14** of the carrier **10**. The spray nozzle **40** may be arranged in an axial orientation with respect to the carrier **10**. The spray nozzles **40** may be arranged in a linear or non-linear array in order to apply individual bands of coating **50**. Each band of coating may extend circumferentially or longitudinally around the carrier **10**, depending on the arrangement of the spray nozzles **40**. For example, FIG. 5 shows a carrier **10** on which a coating **50** has been partially applied.

The spray nozzles **40** may be arranged in a linear array along the length of the carrier **10**, parallel to the axis (A), and thus each spray nozzle **40** may apply a band of coating **50** around the circumference of the carrier **10** as the carrier is rotated around its axis (A) in the direction of arrow (B). Alternatively, the spray nozzles **40** may be arranged circumferentially around the carrier **10** so that each spray nozzle **40** lays down a band of coating **50** along the length of the carrier **10**. The bands may be non-contiguous, leaving parts of the carrier **10** uncoated, or contiguous so that an uninterrupted coating **50** is applied to the carrier **10**. The bands may be any suitable width.

The controller **210** is operably connected to the plurality of spray nozzles **40** to control the operation of the nozzles **40**. For example, the controller **210** may turn the spray nozzles **40** on and off in response to operator input, time, or sensors that sense when the coating has been applied and communicate that information to the controller **210**.

#### EXAMPLES

Experimental tests were conducted on substrates coated with various coatings at various concentrations. The results are summarized in Table 1 below.

TABLE 1

| Example | Agent                                      | Solvent     | Majer Rod | COATINGS                |      | Contact angle, deg. |
|---------|--------------------------------------------|-------------|-----------|-------------------------|------|---------------------|
|         |                                            |             |           | Substrate               | Dyne |                     |
| Control | 0                                          | 0           | #18       | Parchment               | 67   | 34                  |
| 1       | 15% fluorourethane copolymer               | 85% Acetone | #18       | parchment               | 42   | 86                  |
| 2       | 20% fluorourethane copolymer               | 80% Acetone | #18       | parchment               | 42   | 89                  |
| 3       | 10% silicone resin                         | 90% IPA*    | #18       | parchment               | 40   | 109                 |
| 4       | 4% Fluoroalkyl acrylate copolymer emulsion | 96% water   | #6        | parchment               | 30   | 98                  |
| 5       | 4% Fluoroalkyl acrylate copolymer emulsion | 96% water   | #10       | parchment               | 29   | 101                 |
| 6       | 4% Fluoroalkyl acrylate copolymer emulsion | 96% water   | #14       | parchment               | 31   | 93                  |
| 7       | 4% Fluoroalkyl acrylate copolymer emulsion | 96% water   | #18       | parchment               | 28   | 102                 |
| 8       | 10% silicone resin                         | 90% IPA     | #10       | parchment               | 31   | 95                  |
| 9       | 10% silicone resin                         | 90% IPA     | #14       | parchment               | 27   | 105                 |
| 10      | 10% silicone resin                         | 90% IPA     | #18       | parchment               | 29   | 100                 |
| 11      | 4% Fluoroalkyl acrylate copolymer emulsion | 96% water   | #6        | Clay coated kraft paper | 30   | 98                  |
| 12      | 4% Fluoroalkyl acrylate copolymer emulsion | 96% water   | #10       | Clay coated kraft paper | 29   | 101                 |
| 13      | 4% Fluoroalkyl acrylate copolymer emulsion | 96% water   | #14       | Clay coated kraft paper | 31   | 93                  |
| 14      | 4% Fluoroalkyl acrylate copolymer emulsion | 96% water   | #18       | Clay coated kraft paper | 28   | 102                 |
| 15      | 4% silicone resin                          | 96% IPA     | #6        | Clay coated kraft paper | 29   | 101                 |
| 16      | 4% silicone resin                          | 96% IPA     | #10       | Clay coated kraft paper | 31   | 95                  |
| 17      | 4% silicone resin                          | 96% IPA     | #14       | Clay coated kraft paper | 27   | 105                 |
| 18      | 4% silicone resin                          | 96% IPA     | #18       | Clay coated kraft paper | 29   | 100                 |

A fluorourethane copolymer was dissolved in acetone at 15% copolymer /85% acetone and at 20% copolymer/80% acetone. The solution was applied to parchment paper substrate using a #18 Majer Rod. Similarly, a silicone resin was dissolved in isopropyl alcohol (IPA-98.9% pure) at 10% concentration of the silicone resin and applied to a parch-

ment paper substrate. The coated substrates were submitted for surface energy characterization, a key indicator of barrier properties.

#### Contact Angle and Surface Energy Testing

A KRÜSS Mobile Surface Analyzer was used to digitally measure contact angle of water drops (1.0  $\mu\text{L}$ ) applied to the sample surface. The Surface Free Energy was calculated using the ORWK model. The instrument and software were configured in accordance with ASTM D5946. Ten measurements were taken from each variable. A high contact angle will indicate low wettability or high barrier properties.

#### Dyne Testing with AccuDyne Test™ Solutions per ASTM D2578

Dyne testing was performed by first selecting the lowest-numbered dyne solution. A clean cotton-tipped swab was dipped in the solution. A line was wiped onto the test material with the moistened swab. If the mark stayed wetted, i.e. did not bead up, for more than 3 seconds, the procedure was repeated with higher numbered solution until a mark was made that did bead up, shrink, or form a single line in 2 to 3 seconds. The dyne level of this solution was recorded. If the mark beaded very quickly, the dyne level of the solution was considered too high. The lower the dyne level measured, the higher the barrier properties are, indicating poor wettability.

TABLE 2

## EXAMPLES 1-3

| Example | Dyne Solution -<br>dynes | Contact Angle,<br>degrees | Surface Free<br>Energy<br>(calculated<br>from Contact<br>Angle), dynes |
|---------|--------------------------|---------------------------|------------------------------------------------------------------------|
| Control | 67                       | 34                        |                                                                        |
| 1       | 42                       | 86                        | 34                                                                     |
| 2       | 42                       | 89                        | 34                                                                     |
| 3       | 40                       | 109                       | 21                                                                     |

From the results shown on Table 2 it can be seen that the application of the solutions on the parchment result in a lower surface energy/higher contact angle, confirming a less wettable, more water resistant, parchment surface than the untreated control.

## Examples 4-10

A Fluoroalkyl acrylate copolymer emulsion was dissolved in water at 4% Fluoroalkyl acrylate copolymer emulsion/96% water. The solution was applied to parchment paper substrate using a graduated series of Majer Rods. Similarly, a silicone resin was dissolved in isopropyl alcohol (IPA-98.9% pure) at 4% concentration of the silicone resin and applied to a parchment paper substrate using a series of Majer rods. These coated substrates were submitted for surface energy characterization via Dyne Solutions and Contact Angle. Surface energy is a key indicator of wettability and/or barrier properties.

#### Contact Angle and Surface Energy Testing

A KRÜSS Mobile Surface Analyzer was used to digitally measure contact angle of water drops (1.0  $\mu\text{L}$ ) applied to the sample surface. The Surface Free Energy was calculated using the ORWK model. The instrument and software were configured in accordance with ASTM D5946. Ten measurements were taken from each variable. A high contact angle will indicate low wettability or high barrier properties.

#### Dyne Testing with AccuDyne Test™ Solutions per ASTM D2578

Dyne testing was performed by first selecting the lowest-numbered dyne solution. A clean cotton-tipped swab was dipped in the solution. A line was wiped onto the test material with the moistened swab. If the mark stayed wetted, i.e. did not bead up, for more than 3 seconds, the procedure was repeated with higher numbered solution until a mark was made that did bead up, shrink, or form a single line in 2 to 3 seconds. The dyne level of this solution was recorded. If the mark beaded very quickly, the dyne level of the solution was considered too high. The lower the dyne level measured, the higher the barrier properties are, indicating poor wettability.

From the results shown in Table 1 it can be seen that the surface energy, as measured by the contact angle method, generally decreased with higher application rates, for both solutions applied on the parchment substrate. This is shown by higher contact angles when using a higher number Majer Rod. The surface energy as measured by the Dyne Level method, also decreased with higher application rates, for both solutions applied on the parchment substrate. The Dyne Level obtained with higher application rates is lower than the Dyne Level obtained with lower application rate.

## Examples 11-18

A Fluoroalkyl acrylate copolymer emulsion was dissolved in water at 4% Fluoroalkyl acrylate copolymer emulsion/96% water. The solution was applied to a clay coated 35 lbs./3000  $\text{ft}^2$  paper substrate using a graduated series of Majer Rods. Similarly, a silicone resin was dissolved in isopropyl alcohol (IPA-98.9% pure) at 4% concentration of the silicone resin and applied to a clay coated 35 lbs./3000  $\text{ft}^2$  paper substrate using a series of Majer rods. These coated substrates were submitted for surface energy characterization via Dyne Solutions and Contact Angle. Surface energy is a key indicator of wettability and/or barrier properties.

The results shown in Table 1 above indicate that the fluoroalkyl acrylate copolymer emulsion provides good barrier properties on the clay coated sheet at different amounts of coating applied using different Majer Rods. Increasing the concentration or amount of the silicone resin applied to the clay coated sheet did not result in large changes in surface energy reduction, as measured by Dyne Level and Contact Angle results.

## Inks with Barrier Properties

It can be advantageous to print an identifier 38 on the outer surface 14 of the carriers 10, especially near the exposed ends 16, to create a "printed" carrier 10. The identifier 38 may be a name, a color, a symbol, a machine readable code or any other suitable identifier 38. For printing the identifier 38 an ink having barrier properties may be used.

Accordingly, in an optional fourth operation, the method 100 of manufacturing a carrier 10 may comprise the additional step 108 of printing an identifier 38 onto the outer surface 14 of the body 12 near one or both of the ends 16. The printing step 108 may be done using ink jet printing or any suitable manner of applying an ink to cylindrical surface.

The printing step 108 may be done before the coating step 106 so that the identifier is coated and thus protected from textile coatings. Alternatively, the printing step 108 may be done after the coating step 106 or even instead of the coating step 106. In such instances the ink should have a stain resistant formulation that incorporates a barrier compound

or chemical, since a potential problem with some inks is the potential color transfer from the ink to the customer product **20**, e.g., wound yarn. This unwanted color transfer may result from the use by textile manufacturers of aggressive chemical formulations in their textiles that can extract the ink contained in the identifier **38** printed on the outer surface **14** of the carrier **10**. By using an ink having barrier properties, the ink can be protected from the chemicals in the wound products and vice versa.

## EXAMPLES

### Aqueous Based Inks With Barrier Properties

The ink used to make the identifier **38** may comprise an aqueous based ink and a barrier compound. The barrier compound comprised perflouroalkyl acrylic copolymers. Fifteen (15) different aqueous based ink formulations, five each for three different barrier mixtures, were created and evaluated for color pick-up by swab testing:

#### Barrier Mixture #1 (20% Active) Compound:

Control: 100% Aqueous based ink

Sample 1: 70% aqueous based ink and 30% barrier compound;

Sample 2: 60% aqueous based ink and 40% barrier compound;

Sample 3: 50% aqueous based ink and 50% barrier compound;

Sample 4: 40% aqueous based ink and 60% barrier compound;

Sample 5: 30% aqueous based ink and 70% barrier compound;

#### Barrier Mixture #2 (20% active) compound:

Control: 100% Aqueous Based Ink

Sample A: 70% aqueous based ink and 30% barrier compound;

Sample B: 60% aqueous based ink and 40% barrier compound;

Sample C: 50% aqueous based ink and 50% barrier compound;

Sample D: 40% aqueous based ink and 60% barrier compound;

Sample E: 30% aqueous based ink and 70% barrier compound;

#### Barrier Mixture #3 (20% Active) Compound:

Control: 100% Aqueous based ink

Sample I: 70% aqueous based ink and 30% barrier compound;

Sample II: 60% aqueous based ink and 40% barrier compound;

Sample III: 50% aqueous based ink and 50% barrier compound;

Sample IV: 40% aqueous based ink and 60% barrier compound;

Sample V: 30% aqueous based ink and 70% barrier compound;

All fifteen samples demonstrated improved ink smear/stain resistance over the control. In a separate test, an ink comprising 90% aqueous ink and only 10% barrier compound demonstrated improved ink smear/stain resistance over a control lacking any barrier compound.

### Solvent Based Inks with Barrier Properties

Alternatively, the ink used to make the identifier **38** may comprise a solvent based ink and a barrier compound.

Twelve (12) different solvent based ink formulations were created and evaluated for color pick-up by swab testing. In six of the twelve examples, a barrier compound was mixed

with a water based ink. In six other examples, a barrier compound was mixed with a solvent (oil) based ink.

The barrier compound was a perflouroalkyl acrylic copolymer barrier coating, diluted in methanol to achieve a 1%, 2% or 10% active level.

In each case a barrier compound was diluted with methanol to create a barrier mixture, then mixed with the solvent based ink at a rate of 5 parts ink to 1 part barrier mixture to create the ink formulation. The ink formulation was applied to a paper substrate using a cotton swab to create a coated paper. The coated paper was then swabbed with textiles having different chemistries to determine color pick-up, and thus the barrier properties of the ink mixture.

TABLE 3

|                           | SWAB TESTING OF WATER AND SOLVENT BASED INKS WITH BARRIER PROPERTIES |              |              |               |
|---------------------------|----------------------------------------------------------------------|--------------|--------------|---------------|
|                           | Ink Only<br>(No barrier)                                             | 1%<br>Active | 2%<br>Active | 10%<br>Active |
| 60% water based chemistry | 3                                                                    | 2            | 2.5          | 3             |
| 80% water based chemistry | 3                                                                    | 2            | 1.5          | 2             |
| Heavy oil based chemistry | 2                                                                    | 1.5          | 2            | 1.5           |
| Oil base chemistry        | 1.5                                                                  | 2            | 1.5          | 1             |

A lower swab score indicates lower color pick-up, which is desirable. Of the six water based samples tested, five demonstrated lower color pick-up, and thus improved ink smear/stain resistance, over the control. Of the six solvent (oil) based samples tested, three demonstrated lower color pick-up, and thus improved ink smear/stain resistance, over the control.

## INDUSTRIAL APPLICABILITY

Thus, it is possible to achieve a desired barrier level for a paperboard core at least in part by coating the paperboard core **10** with a coating **50** comprising a silicone resin in a solvent and little or no water. An advantage of this coating **50** and method is that the coating **50** does not need to be heat cured. Variables such as the thickness of the coating **50** may affect the barrier properties, and hence may be adjusted in order to obtain the desired properties of the paperboard core.

It also is possible to achieve a paperboard core bearing a printed identifier by using an ink comprising a barrier compound. By using an ink having barrier properties, the ink can be prevented from transferring to the wound product, and chemicals in the wound product can be prevented from transferring into the ink.

It should be understood that the embodiments of the invention described above are only particular examples which serve to illustrate the principles of the invention. Modifications and alternative embodiments of the invention are contemplated which do not depart from the scope of the invention as defined by the foregoing teachings and appended claims. It is intended that the claims cover all such modifications and alternative embodiments that fall within their scope.

The invention claimed is:

1. A paperboard carrier suitable for use in winding a material thereon, the carrier comprising:

one or more strips of paperboard secured together to form an elongate structure, the elongate structure defining an outer surface; and

**11**

a non-aqueous coating disposed on the outer surface in a predetermined region, the coating comprising a coating agent and a solvent, wherein:

the coating is not heat cured.

2. The paperboard carrier of claim 1, wherein: the coating agent is selected from the group consisting of a fluorourethane copolymer, a silicone resin and a fluoroalkyl acrylate copolymer emulsion; and the solvent is selected from the group consisting of acetone, methyl alcohol and isopropyl alcohol. 10

3. The paperboard carrier of claim 2, wherein: the coating consists essentially of the coating agent and the solvent.

4. The paperboard carrier of claim 1, wherein: the coating agent is a fluorourethane copolymer; and the solvent is acetone. 15

5. The paperboard carrier of claim 4, wherein: the coating comprises about 10% to about 20% fluorou- 20 rethane copolymer and from about 80% to about 90% acetone.

6. The paperboard carrier of claim 1, wherein: the coating agent is a silicone resin; and the solvent is isopropyl alcohol.

7. The paperboard carrier of claim 6, wherein: the coating comprises about 4% to about 10% silicone 25 resin and from about 90% to about 96% isopropyl alcohol.

8. The paperboard carrier of claim 6, wherein: the silicone resin comprises a siloxane.

9. The paperboard carrier of claim 6, wherein: the silicone resin comprises silicone resin and octameth- 30 ylcyclotetrasiloxane.

10. The paperboard carrier of claim 6, wherein: the silicone resin comprises about 50% silicone resin and 35 about 50% octamethylcyclotetrasiloxane.

**12**

11. The paperboard carrier of claim 1, wherein: the coating agent is a fluoroalkyl acrylate copolymer emulsion; and the solvent is methyl alcohol.

12. The paperboard carrier of claim 1, wherein: the coating comprises about 50% fluoroalkyl acrylate copolymer emulsion and about 50% methyl alcohol.

13. The paperboard carrier of claim 1, wherein: the coating agent is a reactive silicone resin that produces a durable moisture barrier when the coating is applied to the outer surface.

14. The paperboard carrier of claim 1, wherein: the coating is a predetermined color that identifies a type of carrier.

15. The paperboard carrier of claim 1, wherein: the coating is a spray coating.

16. The paperboard carrier of claim 1, wherein: the predetermined region is one or more annular bands.

17. The paperboard carrier of claim 16, wherein: the one or more annular bands are arranged contiguously such that the coating is uninterrupted.

18. The paperboard carrier of claim 1, wherein: the elongate structure has two ends; and the predetermined region is one or more circumferential bands proximate one or both ends.

19. The paperboard carrier of claim 1, wherein: the material is a textile having a textile coating; and a concentration of the coating agent in the solvent is a function of the textile coating.

20. A carrier suitable for use in winding a material thereon, the carrier comprising:

an elongated tubular body having two ends and defining an outer surface; and a non-aqueous, fast curing, room temperature air dried coating disposed on the outer surface in a predetermined region, the coating comprising a coating agent and a non-aqueous solvent.

\* \* \* \* \*